

Feb. 12, 1957

R. B. HARRISON ET AL

2,780,879

STIFFENING OF SHOE UPPERS AND STIFFENING ELEMENTS THEREFOR

Filed Nov. 16, 1953



1

2,780,879

**STIFFENING OF SHOE UPPERS AND STIFFENING ELEMENTS THEREFOR**

Raymond B. Harrison, Arlington, and Russell G. Edwards, Quincy, Mass., assignors to Stedfast Rubber Company, Inc., Boston, Mass.

Application November 16, 1953, Serial No. 392,302

2 Claims. (Cl. 36—46.5)

This invention relates to the stiffening of a portion of the upper of a shoe. More particularly, it pertains to means and procedure by which a stiffening blank containing a rubber composition can be maintained limp during the upper assembly and shoe lasting operations and become fully vulcanized in lasted shape to a permanently resilient condition while in the finished shoe and before wear.

The invention is applicable to box toes, counters, and other similar stiffening elements. It may best be understood by describing its application to box toes for which it has been employed with outstanding success.

Self-conforming box toes are generally classified as "rigid" and "soft." The rigid type includes all kinds, whether thermoplastic, or solvent activatable, or water activatable, that produce firm toe walls and dome portions upon dissipation of the activating medium used to soften the box toe blank to a condition of workable plasticity directly before shoe lasting operations. The "soft" types comprise all box toes that do not ultimately become fully rigid in the shoe. They embrace a wide range of commercial box toe sheet materials providing a variety of degrees of softness or flexibility for the shoe manufacturers' choice. They are described by the shoe industry as "soft," "semi-soft," "flexible" and "semi-flexible" in order to classify these many box toe materials by the end character of the lasted toe in terms of specific degrees of resilience. The degrees of resilience vary with the box toe material itself, the latex or other cement used to attach the box toe to shoe parts, and the cementing technique used. The range extends from a lifeless softness to a degree of firmness just short of rigidity, and considered flexible only by reason of the yielding of the dome and wall portions to thumb pressure to an extent sufficient to locate the toes of a wearer within the shoe.

All "soft" box toes, except certain light weight pyroxylin types that are self-adhering upon activation by solvent, must be cemented into the shoe upper. Various cements are employed for this purpose and the cementing techniques vary widely in accordance with the value of the shoe and the personal preference of the shoe manufacturer. In most cases, latex cements of natural or synthetic rubber are used to attach the box toe to one or more of its co-engaging shoe parts. In some cases, box toes are cemented on one side with latex and attached thereby to the flesh of the leather upper in the stitching room, and again cemented on the opposite side at the pulling-over operation to engage and permanently affix the shoe lining thereto. A brush applied, naphtha-rubber cement is often employed for this purpose at the pulling-over operation.

Where box toes are cemented into unlined footwear latex cements are almost universally used in preference to the more viscous naphtha-rubber cements.

These attaching cements have an important bearing on the resilience and strength of the finished lasted box toe. If of proper viscosity, their films aid and support

2

the impregnant used in the box toe itself and their effectiveness in causing the toe to be permanently integrated with the co-engaging shoe parts causes the entire structure of vamp, box toe and shoe lining to become a laminate, thus greatly increasing the box toe wall strength. Many lightweight soft box toes having flannel or other textile bases depend nearly as much upon the films which attach the box toe to the shoe lining and/or shoe vamp as upon the box toe itself for the support given the finished lasted toe.

Box toe sheetings containing either natural or synthetic rubber as the principal component of the impregnant used have always been made either partially or fully vulcanized in their finished state, though the liquid impregnant employed has been either entirely uncured or only partially cured such as in the case when impregnants are constructed from pre-vulcanized latices. Box toes cut from partially vulcanized box toe sheetings do not function in the shoe with any degree of permanence though offering the advantage of being more readily conformable at lasting operations than box toes cut from fully precured sheetings. A fully precured box toe, being non-thermoplastic and being unactivatable by any solvent not injurious to other shoe parts cannot be softened to a condition of limpness or static pliability directly before the shoe lasting operations, and permitted to "set-up" through dissipation of the activating medium as is common practice in preparing rigid box toe types for pulling over and bed-lasting. A fully precured box toe fights the conforming action of the bed-lasting wipers and often develops unsightly pin wrinkles in the exterior wall of the shoe toe.

In all shoes which are toe lasted with latex cement and in which the attachment of the overlasted margin of the toe portion of the upper depends upon the latex cement alone for permanent engagement to the insole, the active resilience of the fully precured box toe attempting to return to unlasted shape often acts instantly to pull away from the partially coagulated cement film applied to the surface of the insole only seconds earlier.

Therefore, while the finished soft box toe shoe would be greatly enhanced by the complete curing of the rubber saturant in the box toe, compromises are usually made in the construction of the box toe material to permit the rubber impregnated box toe material to cooperate with the wiping action of the bed-lasting machine.

Accordingly, the general object of this invention is to improve the wearability and appearance of a shoe by providing it with a box toe or other upper stiffening element embodying fully cured rubber material having a high degree of permanent resilience, and yet at the same time avoiding all problems of conforming such elements to the shoe last and of varying or increasing shoe manufacturing operations, or costs, such as derived from the customary practices followed in incorporating fully cured or partially cured box toes or similar stiffening elements.

In the accomplishment of this general objective there has been developed a shoe stiffening sheet material impregnated with an uncured rubber and a curing agent, from which to cut the skive box toes, counters, and the like for incorporation in the upper of a shoe through the use of various rubber cements containing self-curing, migratory vulcanizing accelerators operative at room temperatures. Particularly advantageous in use and commercially available are the dithiocarbamate type room temperature accelerators. In one special instance to be mentioned the use of the curing agent is unnecessary.

Vulcanization or curing of the impregnant composition does not occur at room temperature until the dithiocarbamate or other accelerator migrates from the adhesive cement into the upper-affixed or last-formed box

toe, thus bringing together the sulphur or a curing agent and the accelerator essential for self-curing of the rubber. Various perfecting agents may be used with the sulphur to enhance the powerful action of the dithiocarbamate on the rate of reaction between rubber and sulphur. The impregnant composition is thus changed physically from a plastic condition to a resilient mass creating a lively rebound in the toe structure.

It is a further and specific object of this invention to provide shoe stiffener sheet material of the character indicated with an auxiliary saturant or coating that will add a different uncured rubber component to the sheet material for preventing "blocking" or welding of the sheet material to itself particularly while being "dinked" or cut. The shoe stiffener sheet material having such an auxiliary saturant or coating for preventing "blocking" or welding is the subject of our copending application Serial No. 629,988, filed December 21, 1956.

These and other features of the invention will be particularized and more fully understood from the following detailed descriptions of preferred embodiments, when taken in connection with the accompanying drawing in which:

Fig. 1 is a plan view of a cut and skived toe stiffener blank formed of the sheet material of this invention;

Fig. 2 is a plan view of the inside of the toe portion of a shoe vamp to which the toe stiffener blank of Fig. 1 has been partially applied in the required position by means of adhesive;

Fig. 3 is a plan view of the outer side of a quarter lining partially covered by a counter stiffening blank, made in accordance with this invention, and adhesively joined thereto;

Fig. 4 is a perspective view of the quarter lining of Fig. 3 with the counter stiffening blank adhesively secured to the outer side thereof, the assembly being partially formed to shape for incorporation in the heel end portion of a shoe;

Fig. 5 is a side view of the toe end portion of a lasted shoe of conventional type welt, partially sectioned to show the last and details of box toe construction;

Fig. 6 is a similar side view of the heel end portion of a lasted shoe of welt construction, sectioned to illustrate details of counter stiffening construction; and

Fig. 7 is a bottom perspective view of a last to which a welt insole has been attached, and in which a lining including upper assembly is having cement manually applied to the lining face of the toe blank immediately prior to the pulling-over operation.

In the drawing, 10 refers to the toe stiffener blank which has a skived edge portion 12, and 20 refers to the counter stiffener blank having a peripheral skived edge portion 22 interrupted by a dart 24 for preforming with a quarter lining 26 by use of stitching 28 as shown in Fig. 4.

The shoe stiffener sheet material from which the toe stiffener blank 10 and the counter stiffener blank 20 are formed may be made of any suitable base material such as carded felt, napped or unnapped woven textiles, paper and the like, although only the use of a preferred flannel yard goods will be described in detail. Entirely suitable finished sheet materials in a desired range can be produced from four basic flannels having yard-to-pound relationships of 4.18, 3.00, 2.35 and 1.60.

In actual practice ideal results have been obtained by the use of two saturations and a final spread coating on one side of the saturated base material. Double saturating appears desirable because it has been found difficult to obtain the ounce load required with a single saturation. Further, a second saturation permits the use of a different compound, which, though subject to full curing by the room temperature accelerators contained in the cement, acts to decrease the tendency of the finished stiffener sheet to block to other adjacent sheets, as would occur in packaging and also in cut box toe and counter blanks when die cut in multiple thicknesses on a beam dinker or clicking ma-

chine. Final insurance against blocking is obtained by spread coating a film of the material comprising the second saturating compound on one side of the finished sheet goods. It is possible, however, to obtain adequate impregnation of the saturable base material with only a single saturation of either saturating compound.

An exemplary formula for the first saturating compound is as follows:

*First saturant*

|    |                             | Parts by Weight | Trade Names |
|----|-----------------------------|-----------------|-------------|
| 10 | Crude Rubber (smoked sheet) | 100             |             |
| 15 | Vulcanized Vegetable Oil    | 10              | Amberex-S.  |
|    | Stearic Acid                | 1               |             |
|    | Sulphur                     | 3.5             |             |
|    | Zinc Oxide                  | 5               |             |
|    | Calcium Carbonate           | 90              | Atomite.    |
|    | Titanium Dioxide            | 15              |             |
|    | Antioxidant                 | 1               | Antox.      |
|    |                             | 225.5           |             |
| 20 | Petroleum Naphtha           | 200             |             |
|    | Denatured Alcohol           | 6               |             |

In the above formula, which is a preferred one, the vulcanized vegetable oil may range from 10 to 20 parts, the sulphur from 2 to 3.5 parts, the zinc oxide from 5 to 10 parts, and the inert calcium carbonate particles from 30 to 150 parts. GR-S synthetic rubber (butadiene-styrene copolymer) may be used in place of the crude rubber providing the sulphur is increased to 4.5 to 5 parts.

It will be noted that the above compound includes, in addition to sulphur and other vulcanizing agents, a predominant amount of crude rubber and a very substantial portion of calcium carbonate which acts as a filler. Other rubbers may be employed in the unvulcanized form.

This first saturating compound may be made by premas- tinating the crude rubber on a rubber mill and thereafter adding the other solid ingredients until all are uniformly milled together. Using the petroleum naphtha as a solvent for the rubber and denatured alcohol as a viscosity reducer, the milled material is finally churned to a viscosity suitable for saturation.

The second saturating compound which is used also as a final spreading compound differs in that the predominant elastomeric component is an unvulcanized synthetic rubber which is a rubbery copolymer of butadiene and acrylonitrile. This compound, an exemplary formula of which is as follows, also contains a substantial portion of a resinous copolymer of styrene and butadiene:

*Second saturant and spreading compound*

|    |                                               | Parts by Weight | Trade Names   |
|----|-----------------------------------------------|-----------------|---------------|
| 55 | Synthetic Butadiene (Acrylonitrile Elastomer) | 100             | Paracil B. J. |
|    | Zinc Oxide                                    | 10              |               |
|    | Sulphur                                       | 3.5             |               |
|    | Styrene-Butadiene Copolymer                   | 35              | Marbon 8000.  |
|    | Calcium Carbonate                             | 70              | Atomite.      |
|    | Stearic Acid                                  | 1               |               |
|    | High Melting Synthetic Wax                    | 4               | Aerawax C.    |
| 60 | Titanium Dioxide                              | 15              |               |
|    | Antioxidant                                   | 1               |               |
|    |                                               | 239.5           |               |
| 65 | Toluol                                        | 250             |               |

In the preceding formula, which is a preferred one, the zinc oxide may range from 2 to 10 parts, the sulphur from 2.5 to 3.5 parts, the styrene-butadiene copolymer from 10 to 35 parts, the calcium carbonate from 20 to 70 parts, the stearic acid from 1 to 2 parts, and the wax from 4 to 6 parts.

In this instance the compound may be produced by permatinating the synthetic butadiene elastomer on a rubber mill, and then adding all other solid components until a uniformly milled condition is obtained. Employ-

ing toluol as a solvent, the milled material is churned to a suitable saturating or spreading viscosity.

It has been found that an entirely satisfactory shoe stiffening blank material is obtained by saturating and coating a 1.60 double-napped flannel with the above compounds in the following manner: The flannel is saturated with the saturant of the first compound, and thereafter it proceeds through a drier having a temperature of the order of 180° F. The thus dried saturated material in rolled form is then fed to the second saturant, after which it also travels through a drier having a temperature of the order of 180° F. This roll of dried, double saturated base material is then fed through a knife spreader, which imparts a light coating to one surface only, using the same compound employed in the second saturating treatment. The spreading operation is continuous and the base material coated with the spreading compound proceeds through a drying zone having a temperature of the order of 190° F.

The room temperature, ultra-accelerators that will ultimately contact the surface of the finished box toes, counters, and like shoe stiffening elements will cure both the natural and synthetic rubbers of the two saturating compounds. The particular reason for using the crude rubber impregnant first is that more "bounce," as a characteristic of the finished box toe, develops from the finally cured crude than from the finally cured synthetic rubber. The uncured crude rubber, however, is slightly tacky and prone to weld or block to itself. By using it as a first impregnant and then covering it with the second impregnant comprising a synthetic rubber which, though curable, has much less tendency to weld in its uncured state, welding of either uncured sheet goods or uncured cut shoe stiffener blanks is successfully avoided. It is possible also to use only the second saturant compound by following the previously described procedure with the second saturant compound used for each impregnation. The resulting cured box would have moderately less "life" and bounce as compared to one embodying the crude rubber saturant. In this connection it will be recalled that the shoe stiffening, sheet material will in each instance remain uncured until it is incorporated into the shoe with accelerator-laden cement.

It has been found that an ideal latex cement can be made from the following exemplary formula:

|                                                                    | Parts by Weight | Trade Names                  |
|--------------------------------------------------------------------|-----------------|------------------------------|
| Natural latex (60% solids).....                                    | 167.0           |                              |
| Potassium Hydroxide.....                                           | 0.5             |                              |
| Water-dispersible vulcanizing accelerator (a dithiocarbamate)..... | 30.0            | Setsit-5 (R. T. Vanderbilt). |
| Water.....                                                         | 65.0            |                              |
|                                                                    | 262.5           |                              |

In the above preferred formula the accelerator may range from 20 to 40 parts, and the total water from 40 to 80 parts.

The latex cement compound of the foregoing formula is produced by first dissolving the potassium hydroxide in 5 parts of water, after which it is added to the latex as a stabilizer. The water-dispersible vulcanizing accelerator is then diluted with 60 parts of water and stirred into the balance of the compound.

Since a latex cement is used on the leather engaging side of the stiffening blank, the ultra-accelerator must be dispersible by ball milling or must be water soluble in order to be miscible with the natural latex. Dupont accelerators 89 and "Tepidone" have been tested and found to satisfy these requirements as well as the others involved. "Tepidone" is a 47% water solution of sodium dibutyl dithiocarbamate, according to Dupont.

An entirely satisfactory naphtha-rubber cement has been produced from the following exemplary formula:

|                                                                                                                                                 | Parts by Weight | Trade Names                 |
|-------------------------------------------------------------------------------------------------------------------------------------------------|-----------------|-----------------------------|
| Crude Rubber (smoked sheet).....                                                                                                                | 50              |                             |
| Naphtha.....                                                                                                                                    | 215             |                             |
| Butyl Alcohol.....                                                                                                                              | 6               |                             |
| Vulcanizing Accelerator (a dithiocarbamate containing a slow evaporating liquid; a brown liquid miscible with naphtha and toluene cements)..... | 25              | Butyl 8 (R. T. Vanderbilt). |
|                                                                                                                                                 | 296             |                             |

It is permissible to use from 15 to 30 parts of the accelerator in the above formula.

Denatured alcohol may also be used in the above formula.

The foregoing naphtha-rubber cement compound is produced by masticating crude rubber on a cold rubber mill, after which the batch is put into solution with a petroleum naphtha having a distillation range of 204-220° F. and a Kauri-Butanol index of 45. A closed churn is used for this purpose to prevent solvent loss. The vulcanizing ultra-accelerator is added after the cement is fully churned to blended smoothness, after which further churning is continued until the vulcanizing accelerator is uniformly mixed throughout the cement which, when finished, should contain 18-19% rubber and have a viscosity of approximately 20,000 centipoises. The similar accelerator of Monsanto, N-2126-A, which is also a brown liquid for addition to solvent cements, may also be used. The solid dithiocarbamate Dupont Accelerator 552 is also suitable, but would have to be milled into the rubber before the cement is made.

Selective use of the two types of cement will depend upon the shoe construction involved. For instance, the latex type will be preferred for attaching box toes to the inner face of the vamp on all unlined footwear, since it is cleaner to handle and will function in cementing machines. In lined footwear, the latex cement can be used on both sides of the box toe with the vamp, box toe and vamp lining all cemented together in the stitching room, or the box toe can be cemented to the vamp with the latex type in the stitching room, with the lining left uncemented to the box toe until the pulling-over operation. There the operator, before pulling the shoe, can manually brush a coat of either the latex or the naphtha-rubber cement over the exposed surface of the box toe, engaging the lining to the wet cement film and causing all three parts to become unitary during the course of ensuing shoe making operations.

The naphtha-rubber cement may be preferred for use at pulling-over since many lined shoes are given a brush coat of rubber cement, called "vamp former," between the vamp and the vamp lining in their side portions, and also directly behind the back edge of the box toe, to help avoid vamp lining wrinkles and to hold the lining against the vamp during shoe wear. The naphtha-rubber cement of this invention will act as a "vamp former" as well as to cause curing of the box toe. Thus, the brush coating of the vamp and the coating of the box toe can be accomplished with a single cement in a single work step of the operator, as opposed to using the latex type cement to coat the box toe and a vamp forming cement to unite vamp and vamp lining rearward of the box toe.

It is to be understood that either the latex type or the naphtha-rubber type cement will cure the box toe, and the latex may be used on one side of the box toe and the naphtha-rubber on the other. It will be apparent that the vulcanization of the rubber components of the box toe will occur more rapidly if the curing media is migrating into the box toe from both sides. The box toe cemented with the latex type cement alone, as used in an unlined shoe, will vulcanize more slowly, though as completely,

as box toes in lined footwear having either cement on both surfaces.

Adhesion of the box toe material to the vamp lining is of a character to indicate that the adhesive itself becomes vulcanized, even though it contains no curing agents except the accelerator. It is thought that enough sulphur may be present at the interface to cure the thin adhesive film.

The practice of the shoemaking method involved in the use of the impregnated toe stiffening blank 10 of this invention is specifically illustrated in Figs. 1, 2, 5 and 7. The prepared and skived blank 10 having an adhesive coating 14 of active latex rubber cement containing a room temperature curing ultra-accelerator is positioned and applied to the inner surface of the cut shoe vamp 30. Subsequently an upper assembly including a lining 32 as well as the vamp 30 and adhered toe stiffener blank 10 are placed over the toe end of a last L having a welt insole 34 secured to the last bottom. Thereupon the operator turns back the toe end part of lining 32 and applies an adhesive coating 16 of naphtha-rubber cement containing a room temperature curing ultra-accelerator to the face of the blank 10 engageable by the lining. With the lining 32 adhered to the toe blank 10, the upper assembly is drafted over the last on a pulling over machine and subsequently finally conformed on a bed lasting machine, and the marginal edge portions of the lining, blank and vamp 30 are secured to the welt insole 34, thus conforming the toe stiffener to the last L as shown in Fig. 5.

It will now be fully understood that by reason of the room temperature curing accelerators used as components of each of the two types of cement, and the action of such accelerators on the sulphur contained in the box toe or other stiffening element material when brought into mutual contact or migrating relation when the cement is applied to the box toe or other stiffening element, cause the lasted box toe or other stiffening element progressively to vulcanize to as complete a cure-state as would have been obtained in the event that the impregnated sheet material had been cured before the box toe or other upper stiffening element were cut therefrom. Since the novel sheet material of this invention is uncured, though latently curable through the presence of sulphur in its impregnant, no resistance is offered to the conforming action of lasting equipment. In uncured condition, the shoe stiffeners are limp and extensible, and shape readily to the last. Depending upon whether the cement and its curing accelerators are presented to one or both sides of the stiffener blank, the cure is progressive to a final end point in from 10 to 15 days. This is clear evidence that no degree of immediate cure, consistent with the production speeds of normal shoe manufacturing practice, can impair the susceptibility of the box toe to shoe lasting operations.

The shoe stiffening material of this invention also has excellent adaptability for stiffening the rearward portion of a shoe upper in the region where a molded counter is normally used. Consistent with the increasing demand for "flexible" box toes, there is a growing interest in "soft" or "flexible" heel end structures, particularly for juvenile footwear.

With specific reference to Figs. 3, 4 and 6, it has been found that a very satisfactory result in this direction can be obtained by cutting the quarter lining blank 26 from leather or imitation leather material and cementing with either the latex or naphtha-rubber vulcanizing cement hitherto disclosed the blank 20 of stiffening material that has been suitably skived around its marginal edges, to the inner face of the quarter lining blank in the region to be stiffened, assembling the unitary quarter lining and stiffening blank into the shoe upper 30 by stitching it in place in the usual manner, and thereafter, before the assembling operation in the lasting room, brush coating the inner and previously uncemented surface of the stiff-

fening material with the naphtha-rubber cement to cause the vulcanization of the rubberous saturant contained therein to occur from both surfaces of the stiffening material blank 20.

5 In a variation of this method the stiffening blank would be cemented in position on the quarter itself, and directly thereafter the quarter lining would be cemented to the stiffening blank to produce a unitary construction of three parts before the unit becomes attached to the vamp 10 to form a completed upper. It has been found that the latex type cement is preferable in this procedure.

In a still further variant, satisfactory results can be obtained by merely dipping the cut and skived stiffening blank into the latex type cement and inserting it into the 15 pocket formed by the bottom free and open common marginal edges of the quarter and quarter lining. The cement securely anchors the blank in place and the vulcanizing action proceeds as heretofore described.

As in the case of the box toes, the shaping and conforming action of shoemaking operations will cause the counter blank stiffening element as well as the shoe upper to correspond to the contours of the heel end portion of the shoe last. Having been thus self-conformed, the ultimate self-curing attained will cause preservation of the 20 shape imparted by the dwell on the shoe last. It will be readily appreciated that the counter portions of shoes stiffened in this manner to a "bouncy" resilience afford great comfort to growing feet since there is no rigid encasement of the upper portion of the heel bones to 25 restrict foot growth, and no hard, knife-like edges to abrade against the wearer's foot with resulting discomfort. The complete vulcanization of the rubber components of the stiffening material, coupled with its complete conformability in an uncured state is particularly 30 beneficial in this additional utilization. The contours 35 essential to the character of the heel portion of the shoe are preserved without progressive collapse and fatigue of the stiffening medium that occurs when rubber stiffening blanks are used in an either completely uncured or only partially vulcanized condition.

The term "rubber" as used broadly herein comprehends synthetic as well as natural rubber.

Where in the specification and claims reference is made to "room temperature curing accelerators of the dithiocarbamate type" it is specifically intended to include all dithiocarbamate-producing compounds such as those xanthates that when used with an amine form a dithiocarbamate, in addition to the commercial dithiocarbamate accelerator described in the material relating to the specific examples of adhesive-containing accelerators.

In the formulas set forth herein satisfactory results are obtainable when any combination from the ranges specified is utilized.

The scope of this invention is further demonstrated 55 by the proven fact that a neoprene saturant will cure at room temperature without the use of a curing agent in the saturant by the migration of an xanthate contained in the adhesive.

60 The following formulas have been used successfully:

#### Saturant

|                                        | Parts by Weight | Trade Names |
|----------------------------------------|-----------------|-------------|
| 65 Neoprene (chloroprene polymer)..... | 100             | Type A.C.   |
| Calcium Carbonate (filler).....        | 50              |             |
| High Napthenic Oil (softener).....     | 8               |             |
|                                        | 158             |             |
| 70 Toluol (solvent).....               | 200             |             |

Note: The neoprene is milled with the calcium carbonate and napthenic oil until completely blended whereafter the compound is churned in toluol until a smooth saturable solution is achieved.

9  
Cement

|                                                                            | Parts by Weight | Trade Names                |
|----------------------------------------------------------------------------|-----------------|----------------------------|
| Natural Rubber (smoked sheets)                                             | 100             | ZBX Naugatuck Chemical Co. |
| Zinc Dibutyl Xanthate (a room temperature ultra-accelerator curing medium) | 25              |                            |
|                                                                            | 125             |                            |
| Petroleum Naphtha (solvent)                                                | 220             |                            |
| Butyl Alcohol (viscosity reducer)                                          | 6               |                            |

Note: The above cement is produced by masterbatching 50 parts of premasticated natural rubber with 50 parts of ZBX whereafter the compound is constructed by using 50 parts of the master batch with 75 parts of milled natural rubber resulting in a total of 100 parts rubber to 25 parts of ZBX. The final compound is then churned in 220 parts of the petroleum naphtha (type 2220, having a distillation range of 204-220 deg. and a Kauri-Butanol index of 45). The butyl alcohol is then added, causing the cement to achieve a desired viscosity.

It has been further discovered that a neoprene saturant containing a curing agent can also be cured at room temperature by utilizing the migration of an aldehyde amine accelerator contained in the adhesive.

The formulas which follow exemplify such a modification of curing action:

## Saturant

|                                      | Parts by Weight | Trade Names |
|--------------------------------------|-----------------|-------------|
| Neoprene (chloroprene polymer)       | 100             | Type GN.    |
| Calcium Carbonate (filler)           | 40              |             |
| Light Calcined Magnesia (stabilizer) | 4               |             |
| Litharge (curing agent)              | 5               |             |
| High Naphthenic Oil                  | 8               |             |
| Toluol                               | 157             |             |
|                                      | 200             |             |

Note: The compounding of the above formula is accomplished in identical fashion to the description given in the immediately prior saturant formula.

## Cement

## Cement

|                                                                                                                   | Parts by Weight | Trade Names              |
|-------------------------------------------------------------------------------------------------------------------|-----------------|--------------------------|
| Neoprene (chloroprene polymer)                                                                                    | 100             | Type AC.                 |
| Coumarone-Indene Resin (tackifier)                                                                                | 12              |                          |
| Calcium Carbonate (acid acceptor)                                                                                 | 10              |                          |
|                                                                                                                   | 122             |                          |
| Toluol (solvent)                                                                                                  | 240             |                          |
| Butyraldehyde-Aniline condensation product (a room temperature, ultra-accelerator curing media for neoprene only) | 30              | Accelerator 808— Dupont. |

## 10

Note: Accelerator 833 which is a butyraldehyde-monobutylamine condensation product, also a migratory room temperature ultra-accelerator curing medium, and also a Dupont product may be substituted for Accelerator 808 at equal parts by weight.

Either single or multiple applications of the two neoprene saturants can be made.

The advantages attained through the use of the stiffening blank material of this invention are without increase in the cost of shoemaking operations, and are accompanied by such an enhanced superiority of shoe product, that any increase in impregnated blank material and cement costs is more than compensated by satisfaction to the users of such shoes.

It will be understood that variations, changes, and adaptations can be made in the invention set forth without departing from the principles thereof and the scope of the appended claims.

Having thus described our invention, what we claim as novel and desire to secure by Letters Patent of the United States is:

1. A prepared shoe upper for lasting in which a particular portion is provided with a limp, conformable, extensible sheet of saturable base material impregnated with vulcanizable rubber containing a vulcanizing agent and in which all of said rubber is unvulcanized, said vulcanizing agent being present in amount sufficient for subsequent curing of the vulcanizable rubber, and said sheet being adhesively joined to an inner surface of the upper by a rubber-containing cement which includes in its composition a room temperature curing accelerator in amount capable in coaction with the said vulcanizing agent of causing complete curing of the vulcanizable rubber contained in the sheet whereby the shoe in which said upper is incorporated will have a permanent highly resilient stiffening portion.

2. The combination of claim 1 in which the upper includes a lining member to which said sheet is also adhesively joined by a rubber-containing cement.

## References Cited in the file of this patent

## UNITED STATES PATENTS

|           |                |                |
|-----------|----------------|----------------|
| 1,573,978 | Levine         | Feb. 23, 1926  |
| 1,722,967 | Bennett et al. | July 30, 1929  |
| 1,777,544 | Beckwith       | Oct. 7, 1930   |
| 1,831,689 | Swett          | Nov. 10, 1931  |
| 2,197,928 | Finn           | Apr. 23, 1940  |
| 2,201,931 | Sullivan       | May 31, 1940   |
| 2,363,981 | Lissig         | Nov. 28, 1944  |
| 2,512,003 | Wedger         | June 20, 1950  |
| 2,541,748 | Daly           | Feb. 13, 1951  |
| 2,611,195 | Brophy et al.  | Sept. 23, 1952 |
| 2,646,379 | Poschel        | July 21, 1953  |